

## UNITED STATES PATENT OFFICE.

NATHAN R. LEVY, OF CEDARHURST, NEW YORK.

## PLASTIC MATERIAL AND METHOD OF MAKING THE SAME.

No Drawing.

Application filed May 27, 1922. Serial No. 564,232.

*To all whom it may concern:*

Be it known that I, NATHAN R. LEVY, a citizen of the United States, residing at Cedarhurst, in the county of Nassau and State of New York, have invented certain new and useful Improvements in Plastic Materials and Methods of Making the Same, of which the following is a specification.

This invention relates to plastic materials and methods of making the same.

In the present invention, I provide a plastic material by treating a suitable fibrous substance or other filler mixed with a soluble soap of a drying oil with a solution of a metallic salt that will react with the soap to form a water insoluble compound which serves as a binding agent to hold the fibrous material together. The material is then dried, the soap oxidized and the material disintegrated for molding or pressing into the desired shapes.

An object of the present invention is the provision of an improved plastic material for molding or pressing into desired shapes.

A further object is the provision of an improved process for making plastic material by precipitating a soluble soap of a drying oil mixed with suitable fibrous material or other filler to form a water insoluble product.

In performing the process, a mixture of suitable fibrous material, such as cotton, paper pulp, asbestos or the like, or other suitable inert substance, and a solution of a soluble soap of a drying oil, such as sodium linoleate, or other similar substance, is treated with a metallic salt capable of forming a water insoluble compound with the soap of the drying oil to precipitate an insoluble soap in the mixture of fibrous material. This mixture is passed through a beater or other type of agitating machine to thoroughly mix the fibrous material and the insoluble soap is then filtered and the solution drained off. The residue is then disintegrated, dried, and oxidized. This oxidation consists in allowing the insoluble soap of the drying oil to take up its proportion of oxygen and has a reaction substantially similar to the "drying" of a linseed oil paint. It may be hastened by any of the methods ordinarily employed to hasten the drying of paint, such as the circulation of heated air, the use of catalytic agents, and the like. After the oxidation is ap-

proximately completed, the material is removed from the drier and is disintegrated in a mill or disintegrator to form a homogeneous mass. The material is then ready to be molded by heat and pressure into 60 the desired shapes.

In a typical embodiment of the invention, a suitable fibrous material, such as cotton, paper pulp, asbestos or other inert material is disintegrated in water by means of a 65 paper beater or other suitable machine until a pulp of the desired fineness is obtained. A water solution of a soluble soap of a drying oil, such as a soda soap of linseed oil and preferably of "boiled oil" is 70 added to the fibrous material and the beater run for a sufficient length of time, about fifteen minutes, to incorporate the soap in the fibre. A solution of a metallic salt, capable of forming an insoluble soap is 75 then added to the material and the insoluble soap precipitated. Various salts may be employed for this purpose, such as lead nitrate, aluminum sulfate, calcium chlorid and other salts soluble in water and capable 80 of forming an insoluble linoleate.

The beater is then run for a short period of time, less than one-half hour, and the mixed pulp is then run to a filter bed or other suitable device to drain the excess 85 solution. The residue is preferably washed free, or reasonably free of soluble salts formed, such as sodium sulfate, sodium chlorid, and the like, and is then picked apart into small pieces and placed in a 90 drier or other suitable apparatus to dry the material and oxidize the insoluble soap. During the drying process, it is preferable to employ a current of warm air passing through the material to hasten oxidation. 95 Various temperatures may be employed, depending upon the nature of the fibrous material. A temperature up to 100° C., or even higher may be employed under some conditions. After the oxidation is approximately completed, the material is disintegrated in a mill to form a homogeneous mass, and it is then ready to be molded by heat and pressure into desired shapes.

Dyes or pigments may be added to produce 105 objects of desired colors. They may be added to the beater before the addition of the metallic salt or after, depending upon the particular nature of the composition being treated and the nature of the dye 110

added. Pitch or other materials, to give special properties, may be added in the beater or in the mill used after oxidation.

- The process set forth may be varied with-  
5 in wide limits as for instance, the metallic salt may be first added to the fibrous mate-  
rial and the solution of the soap of the dry-  
ing oil added afterward. The proportion  
10 of a soap of a drying oil may be varied  
within wide limits. Under some conditions,  
a very small amount is employed merely  
furnishing a small proportion of oxidized  
material in the mixture, and under some  
15 conditions, the linseed oil or other drying  
oil may be present in excess of that re-  
quired to combine with the metallic salt,  
whereby a more flexible material may be  
produced and one that may be more easily  
20 worked with cutting tools.

- 20 In place of linseed oil, I may employ  
soaps of other drying oils, such as tung oil,  
perilla oil, fish oil and the like.

While I have described in detail the pre-  
ferred practice of my process, it is to be un-  
derstood that the details of procedure, and  
25 proportion of ingredients may be widely  
varied, and that known chemical equivalents  
may be employed in place of the materials  
mentioned, without departing from the  
30 spirit of the invention or the scope of the  
subjoined claims.

Having thus described my invention, I  
claim:

1. A plastic material consisting of a  
35 fibrous substance, and an oxidized insoluble  
soap of a drying oil.
2. A plastic material consisting of a  
fibrous substance, and an oxidized insoluble  
soap of linseed oil.
- 40 3. A plastic material consisting of a  
fibrous substance, and an oxidized metallic  
insoluble soap of a drying oil.
4. A plastic material consisting of a  
fibrous substance, and an oxidized metallic  
45 insoluble soap of linseed oil.
5. The process of making plastic material  
which consists in impregnating a fibrous  
substance with a soluble soap of a drying  
oil, adding a solution of a metallic salt  
50 adapted to form an insoluble compound with

the soap, drying the material, oxidizing the  
precipitated soap contained in the material,  
and disintegrating the material.

6. The process of making plastic material  
which consists in impregnating a fibrous 55  
substance with a soluble soap of linseed oil,  
adding a solution of a metallic salt adapted  
to form a water insoluble compound with  
the soap, drying the material, oxidizing the  
precipitated soap contained therein, and dis- 60  
integrating the material.

7. The process of making plastic mate-  
rial which consists in impregnating a fibrous  
substance with a soluble soap of a drying 65  
oil, adding a solution of aluminum sulfate  
to form an insoluble soap, drying the mate-  
rial, oxidizing the precipitated soap con-  
tained therein, and disintegrating the ma-  
terial.

8. The process of making plastic material 70  
which consists in impregnating a fibrous  
substance with a soluble soap of linseed oil,  
adding a solution of aluminum sulfate to  
form an insoluble soap, drying the material,  
oxidizing the precipitated soap contained 75  
therein, and disintegrating the material.

9. The process of making plastic material  
which consists in impregnating a fibrous  
substance with a soluble soap of a drying  
oil, adding a solution of a metallic salt 80  
adapted to form an insoluble compound with  
the soap, drying the material, oxidizing the  
precipitated soap contained in the material,  
disintergrating the material, and molding  
and pressing it into the desired form. 85

10. The process of making plastic mate-  
rial which consists in impregnating a fibrous  
substance with a soluble soap of linseed oil,  
adding a solution of a metallic salt adapted  
to form an insoluble compound with the 90  
soap, drying the material, oxidizing the pre-  
cipitated soap contained in the material,  
disintegrating the material, and molding  
and pressing it into the desired form.

In testimony whereof, I affix my signa- 95  
ture in presence of two witnesses.

NATHAN R. LEVY.

Witnesses:

L. V. EATON,  
M. R. BHAGWAT.